

## UNITED STATES PATENT OFFICE

2,031,431

## QUENCHING OILS

George Chapelton Shepherd, Jr., Long Beach, Calif., assignor to Union Oil Company of California, Los Angeles, Calif., a corporation of California

No Drawing. Application January 9, 1933,  
Serial No. 650,863

3 Claims. (Cl. 148—18)

This invention relates to quenching oils for use in the metallurgical industries, to methods for their production, and to methods of quenching where these oils are employed.

5 The object of the invention is to furnish quenching oils which will afford greater cooling velocities throughout the critical and tempering stages than heretofore, and which at the same time will not deteriorate materially under the severe service conditions to which said oils are subjected. In the past no quenching oil of high cooling velocity has been known, and many of those available have been subject to great deterioration in use as has been indicated by a resultant thickening and formation of sludge. This has been true particularly of those types including fish and animal oils.

I have discovered that, by employing mineral oils which have been so heat-treated as to be highly resistant to further change by heat, quenching may be efficiently accomplished and deterioration of the quenching oil will be almost entirely eliminated. Such oils are cracked oils of sufficiently low viscosity and volatility as to be suitable for quenching purposes and to afford the desired high cooling velocities. Thus certain fractions suitable for these ends are obtained by the distillation of cracked residuums which have been produced by the well known cracking processes for conversion of petroleum into lighter products, as in the manufacture of motor fuels. Other suitably heavy fractions of cracked distillates also are included. One important advantage of these cracked oils resides in their great fluidity and their high flash points, the flash point being always relatively high and the viscosity relatively low. This high degree of fluidity is conducive to free circulation of the quenching oil about the metal being treated whereby high cooling velocities are induced.

The invention therefore may be stated broadly as covering quenching oils comprising relatively non-volatile cracked fractions of low viscosity obtained from the cracking of mineral oils. The invention particularly includes such fractions where obtained by distillation of cracked mineral oil residuums resulting from the various well known cracking processes, as well as from residuums from other hydrocarbon cracking processes. The invention includes further the methods of manufacturing such quenching oils and methods for quenching metals therewith.

Considering the invention in greater detail, oils which possess the required non-deteriorating

characteristics include particularly those which are recoverable by distillation from residuums from the cracking of hydrocarbons particularly of mineral oils and mineral oil products as in the case of the manufacture of cracked gasoline. 5 These residuums consist largely of complex polymers which have been formed incidental to the cracking processes, and when these polymers are separated as suitable fractions, they are found to present the desired stable properties here considered essential to good quenching oils. In general, the more severe the cracking, the more useful will be the product. Where petroleum and petroleum fractions have been cracked either by liquid phase or vapor phase methods, the residuums or liquid bottoms resulting from the fractionation of the cracked products constitute suitable stocks from which the desired quenching oils may be obtained.

For example, such a stock is the heavy residuum 20 resulting where a gas oil obtained from a California or other asphaltic crude, such as San Joaquin Valley crude, is cracked by means of a cracking process at temperatures around 850 to 900° F. when producing cracked gasoline. This residuum results after removal of the lighter cracked products therefrom. Other residuums which will serve as suitable stocks are those recovered from other cracking operations, particularly severe cracking operations, and in addition to those from the cracking of petroleum liquids or vapors, residuums obtained from the cracking of natural gas or similar hydrocarbons will constitute satisfactory stocks. 35

Having obtained a cracked residuum of the character stated, the residuum itself is then distilled, as by means of steam distillation at atmospheric pressure to separate the oil into fractions of varying volatility. The first fractions, if they have the characteristics of kerosene or light gas oil, will in themselves be too volatile and will therefore be discarded, but the succeeding heavier cuts which possess a sufficiently high flash point will be condensed and blended to produce an oil 45 satisfactory for quenching purposes. Such an oil ordinarily should have a flash point not lower than about 300° F., and for average purposes may for example have a viscosity of around 125 seconds Saybolt universal or less at 100° F. A suitable oil obtained from the San Joaquin Valley gas oil cracked by recycling as above indicated, has a rather wide boiling range and may have been obtained by distilling until the bottoms showed a melting point around 250° F. The 55

lightest fraction will ordinarily have been discarded however as above indicated, and the heavier fractions of proper flash point blended to yield the product. The desirable cracked oil fractions which I employ as the quenching oil are characterized by the property of having a greater density than that of uncracked oils for the same viscosity range. A specific example of a suitable product obtained from the mentioned gas oil is one having a viscosity of 115 seconds Saybolt at 100° F. and an A. P. I. gravity of 7.9° at 60° F., and a flash point of 320° F. In general it may be said that satisfactory oils obtained as indicated probably should have viscosities which lie between about 75 and 200 seconds Saybolt universal at 100° F. and might have flash points as low as 250° F. in some instances. The oil fractions obtained are for the most part within the range of the light lubricating fractions of cracked oil. The characteristics of the quenching oil of the above example having a viscosity of 115 seconds as compared with two other quenching oils in common use are indicated by the fact that in using the oil of the present invention the metal is cooled from a temperature of 1500° F. down to 300° F. in about 190 seconds whereas the other two oils require something over 400 seconds. Thus in employing the oil of the present invention the quenching procedure, which consists in quenching the heated metal in the oil until properly cooled, results in a more rapid cooling, and as previously indicated results in elimination of substantially all thickening and formation of sludge and other deterioration heretofore commonly encountered in the use of quenching oils.

It is to be understood however that both lighter and heavier fractions may be employed, especially for certain uses, so long as the volatility of the products does not exceed that of a safe flash point. Thus, any cracked fraction of sufficiently low volatility and sufficiently low viscosity may be segregated from the overhead or vaporized products obtained in any cracking process. For example, where manufacturing cracked motor fuels, the overhead or vaporized products are ordinarily recovered in the form of a lighter or gasoline fraction and a heavier fraction which is known as "cycle stock" and is returned to the cracking system. By in turn fractionating a quantity of this cycle stock in order to eliminate the lighter and more volatile portions, a heavier cut or liquid bottoms may be taken which will constitute a satisfactory quenching oil possessing the desired high flash point and low viscosity. Again, the above described residuum which is formed when the gasoline and cycle stock cuts are fractionated off, may itself be used as a quenching oil in some cases where a greater viscosity is not objectionable. This would be particularly true when a quenching oil having only moderately high cooling velocities is desired and cheapness is a consideration.

The cracked fractions above described as having suitably low viscosity and volatility may be used as quenching oils without further treatment, or they may be refined by any of the methods customary in refining petroleum products. However the distilled fractions which have been blended to produce an oil suitable for use in quenching, should in general, be chemically treated to remove highly unsaturated and other easily oxidized bodies which would tend to produce sludge during use. The treatment which I have found to be satisfactory, consists in subjecting the oil to the action of sulfuric acid of 98% strength at 100 to 110° F. in the proportion of 25 pounds of acid per barrel of oil. After separating the sludge, the oil is neutralized with a solution of alkali, such as sodium hydroxide, and then water washed. The resulting treated oil may then be blown bright with air at a temperature of 150 to 180° F. and/or may be contacted with decolorizing clay to improve the color. While 98% acid is generally preferable, acids of lower strength as well as fuming acid may be employed.

The above described oils, whether refined or unrefined, present the desired characteristics of high flash point and such fluidity as to circulate freely for rapid cooling when in use. They may be used either alone or as the important components of compounded quenching oils. For example small quantities of animal or vegetable oils may be added as is well understood by those skilled in the art; in a specific instance 15%, or more or less, of fish oil may be added, and other constituents as found advantageous or desirable may be included in the preparation of any particular compound for any special purpose.

It is to be understood that the specific disclosures hereof are not to be taken as limiting but merely as illustrative of the generic invention which relates to the use of any stable cracked product as a quenching oil.

I claim:

1. A method of quenching metals which comprises immersing the heated metal in a heavy cracked hydrocarbon oil fraction, said oil being characterized by having a flash point of 250° F. or higher and a viscosity of between 75 to 200 seconds, Saybolt universal at 100° F.

2. A metal quenching oil comprising a heavy cracked mineral oil fraction having a flash point of 250° F. or higher and a viscosity of 75 to 200 seconds, Saybolt universal at 100° F.

3. A method of quenching metals which comprises immersing the heated metal in a cracked hydrocarbon quenching oil produced by cracking a mineral oil to yield cracked residuum, distilling said residuum and recovering said quenching oil as a heavy condensate characterized by a viscosity of between 75 to 200 seconds Saybolt universal at 100° F.

GEORGE CHAPELTON SHEPHERD, JR.